

## UNITED STATES PATENT OFFICE

VAN M. DARSEY, OF MORENCI, MICHIGAN, ASSIGNOR TO PARKER RUST-PROOF COMPANY, OF DETROIT, MICHIGAN, A CORPORATION OF MICHIGAN

## RUSTPROOFING MATERIAL AND METHOD OF TREATING THE SAME

No Drawing.

Application filed November 15, 1928. Serial No. 319,733.

This invention relates to a rust-proofing material and more particularly to such a material which may be kept in granular or powdered form under usual weather conditions without deterioration. More specifically, the invention relates to a rust-proofing material comprising granular or powdered high acid phosphates with a material added thereto for deterring the drying out of the phosphates.

10 This invention is applicable to rust-proofing material such as that disclosed in the patent to Green et al on rust-proofing, No. 1,651,694, dated December 6, 1927, and which 15 includes phosphates of the metals of the electromotive series from manganese to iron, inclusive, and corresponding substantially to the formula  $M(H_2PO_4)_2$ .

Rust-proofing material such as that disclosed and claimed in the above cited patent 20 contains a certain amount of water when first formed. Some of this is water of crystallization and some of it is doubtless present in other forms. When the freshly formed material is exposed to the air at ordinary temperatures there is generally a slight initial 25 loss of weight by drying and a subsequent absorption of moisture from the atmosphere to equal or exceed the original weight of the 30 material. The freshly formed material is more readily soluble in a rust-proofing bath than is the material after it has dried to this slight extent and then reabsorbed moisture. The appearance of the crystals undergoes a 35 change during this initial loss and subsequent reabsorption of moisture, which can be detected under the microscope, the older crystals being rougher in appearance than those first formed. These differences in the characteristics of the material after initial loss of 40 weight and subsequent reabsorption indicates that there is some difference in the nature of the moisture present, but just what this is cannot be stated at the present time.

45 When material such as that described

above has gone through this initial slight drying stage and subsequent absorption of water, and is exposed to temperatures as high as are generally attained in the United States during the summer time, it frequently 50 cakes to a greater or less extent. This caking does not seem to seriously affect its chemical composition, so that if it is reground it may be used readily for rust-proofing purposes, and with nearly its initial efficiency. But unless it is subjected to a somewhat troublesome process for breaking up the lumps and regrinding it is not as satisfactory 55 for forming a rust-proofing bath, as the lumps dissolve much more slowly and are likely to become covered with sediment before entirely dissolved, so that their solution is never completed. For this reason some 60 means is desirable for preventing such caking and lumping of the material when exposed to summer temperature.

It has been found that this lumping of the material can be effectively prevented by preventing the initial drying of the material. As long as the material is prevented from undergoing 65 this initial drying step, the moisture seems to remain present in its original relation to the crystals and the crystals retain 70 their original characteristics. The material which has been so treated as to retain its 75 original moisture retains also its accompanying original characteristics and not only handles more readily, because it does not undergo lumping, but also is somewhat more readily soluble and, therefore, more efficient as 80 a rust-proofing material.

This initial drying of the material may be prevented by hermetically sealing the material immediately after its formation so as to mechanically prevent the escape of moisture from the container. The drying out 85 may be prevented also by mixing therewith various materials which have the property of retaining moisture. There are many such materials well known, and which, therefore, 90

do not require enumeration. While there are a great many different substances which would accomplish the purpose of retaining the initial moisture of the phosphate crystals and maintaining the material in its original condition, most of these materials are objectionable as adulterants for various reasons.

It will be obvious that if the material does not dissolve in the rust-proofing bath it will necessarily form a sediment which increases with the successive replenishments of the bath, thus adding to the sludge in the bottom of the tank. While this is not an insuperable objection, it is an undesirable feature and one which is to be avoided if conveniently possible.

Of materials which will perform the desired function of retaining moisture and which are soluble at least to some extent in the rust-proofing bath, there are some which are positively injurious to the efficiency of the bath, even in small quantities. Furthermore, any material which is soluble in the bath and which is added repeatedly in the powder used to replenish the bath, tends to increase in the bath until it reaches an objectionable amount, unless there is some way in which it is automatically removed.

Of the materials which have been tried for preventing the lumping of the powder and retaining it in its original condition by preventing its drying out, the most satisfactory are zinc carbonate, sugar and boracic acid. Of these three materials, boracic acid is preferred because it not only is not detrimental to the efficiency of the bath, at least in the small amounts necessary to accomplish the purpose of this invention, but also during the boiling of the solution it volatilizes sufficiently to prevent detrimental building up in the bath. Under ordinary conditions as small an amount of boracic acid as 1% by weight of the phosphate powder effectively prevents the detrimental drying out of the powder. A less amount has some beneficial effects and a greater amount can be used without any noticeable detrimental effect upon the bath. For that reason the exact percentage of boracic acid added to the powder for the purpose of preventing drying out and subsequent lumping may be varied within considerable limits. The practice at present preferred for commercial purposes is the use of from 1 to 3%, but in its broader scope the invention is not limited to this percentage. Also, while boracic acid is the best material thus far discovered, there are other materials, notably sugar and zinc carbonate, which can be used with considerable benefit, and even other materials, less satisfactory from the standpoint of subsequent use in the bath, can be effectively utilized for the purpose of preventing the drying out and caking of the powder. For these reasons various materials in various amounts may be added to the phos-

phate powder for the purpose specified, and come within the scope of the invention as set forth in the appended claims.

Furthermore, while it is preferred to prevent the drying out of the phosphate powder by a material whose chemical composition is such as to accomplish this purpose, the broad method of preventing the caking by preventing drying out may include hermetical sealing as well as chemical prevention of drying out.

What is claimed is:

1. The method of treating rust-proofing material consisting substantially of high acid phosphates of metals of the electromotive series from manganese to iron, inclusive, in granular or pulverulent form, which comprises preventing the drying out of such materials from the time of their formation until they are to be used by dissolving in a rust-proofing bath, and thereby preventing the change in the relation of the water associated with the material and consequent lumping or caking of the material which might otherwise occur. 90

2. The method which consists in forming crystals of high acid phosphate of manganese, separating the crystals from their mother liquor, and thereafter, and before the crystals dry out, mixing therewith boracic acid. 95

3. A rust-proofing material comprising high acid phosphates of metals suitable for forming a rust-proofing bath for iron or steel, and containing a material which deters the drying out of the phosphate and thereby prevents lumping and caking. 100

4. A rust-proofing material comprising crystalline high acid phosphates of metals of the electromotive series from manganese to iron, inclusive, and a material added to the crystals immediately after their separation and adapted to deter the drying out of said crystals. 105

5. A rust-proofing material comprising high acid phosphates of metals of the electromotive series from manganese to iron, inclusive, in granular or pulverulent form and containing boracic acid. 110

6. A rust-proofing material comprising high acid phosphates of metals of the electromotive series from manganese to iron, inclusive, in granular or pulverulent form and from 1 to 3% boracic acid. 115

7. A rust-proofing material comprising high acid phosphates of one of the metals in the electromotive series from manganese to iron inclusive in crystalline form and having, added to said crystals after their formation and before drying out occurs, sufficient boracic acid to deter the drying out of the crystals and a change of the relation of the water to the phosphates resulting in caking or lumping. 120

8. A rust-proofing material comprising manganese dihydrogen phosphate in granu. 130

lar or pulverulent form, and from 1% to 3% of boracic acid.

9. The method which consists in forming crystals of high acid phosphate of manganese, separating the crystals from their mother liquor, and thereafter and before the crystals dry out, mixing therewith boracic acid.

In testimony whereof I have hereunto signed my name to this specification.

10 VAN M. DARSEY.

15

20

25

30

35

40

45

50